

# UNITED STATES PATENT OFFICE.

THEODORE G. TIMEBY, OF CHICAGO, ILLINOIS.

## METHOD OF PRODUCING LEAD HYDRATE.

1,056,382.

Specification of Letters Patent. Patented Mar. 18, 1913.

No Drawing.

Application filed March 2, 1912. Serial No. 681,299.

To all whom it may concern:

Be it known that I, THEODORE G. TIMEBY, a citizen of the United States, residing at Chicago, in the county of Cook and State 5 of Illinois, have invented a certain new and useful Method of Producing Lead Hydrate, of which the following is a specification.

My invention relates to a new and useful method of producing lead hydrate from 10 lead ores, particularly lead sulfid concentrates.

I have discovered that by employing cast 15 lead-bearing ore, in any convenient form such as bars or cakes, as the anode of an electrolytic cell containing a suitable electrolyte dissolved in water, such for example as a neutral solution of sodium nitrate in water, I can quickly and cheaply produce lead hydrate.

20 In practice I prepare bars or cakes of lead bearing ore used as anodes by fusing lead sulfid ore, preferably in a reverberatory hearth in which the atmosphere of the chamber above the ore is kept practically 25 reducing by allowing it to remain full of the gaseous products of combustion from the fire box, and then casting or molding the fused ore into bars or cakes in suitable molds of refractory material. In practice I 30 find that satisfactory results are obtained when these bars or cakes are in the form of slabs approximately eighteen inches long, twelve inches wide and two inches thick, provided with suitable heads for the positive 35 terminal of the usual electric circuit; it is of course understood that these dimensions may be varied. One or more of such anodes are arranged and supported with their bodies immersed in the liquid of an 40 electrolytic cell containing a suitable electrolyte preferably a neutral solution of sodium nitrate in water, and provided with one or more of the usual cathodes. When 45 the cell or apparatus is thus equipped and electric current is passed through the anode in any usual manner and by any suitable means now well known in the art of electrolysis, the cast lead-bearing ore anode is electrolyzed and the liberated lead is spontaneously 50 precipitated as lead hydrate by reaction with the water of the bath. The hydrate may be converted into other compounds, particularly lead carbonate or lead 55 oxids, by suitable treatment.

Preferably I employ iron wire mesh for

the cathode. If the anode and cathode are placed too close together, or if the hydrate produced be allowed to collect on the cathode, considerable metallic lead is produced. By using a low potential, preferably not over four volts, and by placing the anode and cathode approximately three inches apart, the metallic lead is reduced to a negligible quantity. Furthermore, reduction of the hydrate to metallic lead is 60 prevented by placing the cathode in a cloth cell.

By my process all the electricity acts directly upon the cast lead-bearing ore, so that the latter is quickly and cheaply decomposed; and, furthermore, the electrolytic bath is not surcharged with excess of soluble reagents and the same bath can be used for a considerable period, although as the water soluble compounds of the ore and 70 sulfur therefrom gradually accumulate upon the anode within the bath it may be necessary from time to time to renew the solution or to substitute fresh solution.

A unique feature of my process is that the 80 reagents of the bath effect precipitation of the lead hydrate and are regenerated by recombining so that the bath remains unchanged except for the slight loss of water combined in the lead hydrate. This cyclic 85 action effects economy in consumption of chemicals and is illustrated by the following reactions:



Reaction (1) illustrates the dissociation of the sodium nitrate and water into sodium hydrate and nitric acid. Reaction (2) shows the decomposition of the lead sulfid by the nitric acid so produced, the sulfur being deposited and the lead passing into solution as nitrate. Reaction (3) is the decomposition of the nitrate so formed on encountering the sodium hydrate formed in the first reaction with the formation of lead hydrate and the regeneration of sodium nitrate. 105

With a potential between one and six volts the current separates some free sulfur at the anode; this sulfur is not mixed with the hydrate but forms a coating on the anode itself which may be removed by 110

brushing the anode, or when an envelop or diaphragm is used it catches and retains the coating when the latter develops to such thickness that it sloughs or scales off. Only a negligible amount of sulfur is found in the hydrate and this is present wholly as a sulfate of lead which is not detrimental and does not affect the value of the hydrate as it is inert and does not affect the color of any product made from the hydrate.

By my present method of fusing the ore less through oxidation is avoided, and the anode metal is precipitated spontaneously by the water in the electrolytic bath or cell.

I am aware that it has been proposed to employ cast lead-bearing ore anodes in a bath of molten lead compounds such as lead chlorid or lead chloro-sulfid, for the production of molten metallic lead, but such treatment could not produce lead hydrate, and so far as I am aware I am the first to produce by electrolysis lead hydrate, the basis of many valuable lead products.

I claim:—

1. The method of producing lead hydrate which consists in electrolyzing a cast anode of lead sulfid ore in a neutral hydrous solution of a nitrate of an alkaline base, and precipitating the hydrate in the electrolytic

cell by the reaction of the ingredients of the bath.

2. The method of producing lead hydrate which consists in electrolyzing a cast anode of lead sulfid ore in a neutral hydrous solution of sodium nitrate, and precipitating the hydrate in the electrolytic cell by the reaction of the ingredients of the bath.

3. The method of producing lead hydrate which consists in electrolyzing a cast anode of lead sulfid ore in a neutral hydrous solution of a nitrate by a current of low potential, and precipitating the hydrate in the electrolytic cell by the reaction of the ingredients of the bath.

4. The method of producing lead hydrate which consists in electrolyzing a cast anode of lead sulfid ore in a neutral hydrous solution of sodium nitrate by a current of low potential and in the presence of a cathode in a cloth envelop, and precipitating the hydrate in the electrolytic cell by the reaction of the ingredients of the bath.

In testimony whereof I affix my signature in presence of two witnesses.

THEODORE G. TIMBY.

Witnesses:

J. McROBERTS,  
H. C. JUST.